

## UNITED STATES PATENT OFFICE

1,947,656

LEDEBURITIC, PRELIMINARY IRON ALLOY  
FREE FROM GRAPHITEJosef Novak and Roman Kesselring, Novy  
Bohumin, CzechoslovakiaNo Drawing. Application April 12, 1932, Serial  
No. 604,868, and in Germany April 13, 1931

3 Claims. (Cl. 75—1)

The invention in our co-pending application 553681/31, now Patent No. 1,890,540, Dec. 13, 1932, comprises a ledeburitic iron pre-alloy free from graphite, characterized by a chromium content of 20 to 30%, a tungsten content of 5 to 6%, a nickel content of 6 to 10%, a copper content of 10 to 15% and a carbon content of 2½ to 3%. This pre-alloy serves, in the first instant for manufacturing a steel practically free from silicon, that is not over 0.002% and containing chromium 0.1 to 1%, copper 0.25 to 0.50%, nickel 0.04 to 0.25% and tungsten 0.01 to 0.05%.

For the production of steels, which are to contain, besides the above-enumerated metals, chromium, tungsten, nickel and copper, also refining metals, such as zirconium, aluminium, boron, beryllium, molybdenum and titanium singly or in combination, pre-alloys are to be used, which contain both of said groups of metals. 20 Alloys of this character are the object of the present invention.

All these pre-alloys contain iron and the refining metals within the following limits namely: chromium 20 to 30%, tungsten 2 to 6%, nickel 25 6 to 15% and copper 10 to 15%, together with 2½ to 3% carbon, which is present as a carbide combination. The alloys are, consequently, all free from graphite and have a ledeburitic structure.

30 Besides these components, contained in common with the pre-alloy according to the copending application No. 553681, now Patent No. 1,890,540, Dec. 13, 1932, the pre-alloy of the present invention contains also the following refining metals: about 5 to 8% zirconium, 2 to 3% aluminium, 3 to 4% boron, 8 to 10% beryllium, 5 to 18% molybdenum and 1 to 2% titanium.

The refining metals last named may be contained in the present pre-alloy singly or in combination.

Below are stated four modifications of the pre-alloy according to the present invention by way of example, which have proved highly satisfactory:

## Example I

|       | Per cent  |
|-------|-----------|
| Cr    | 20-30     |
| Cu    | 10-15     |
| 50 Ni | 6-10      |
| W     | 2-3       |
| Zr    | 5-8       |
| Mo    | 6-12      |
| C     | 2½-3      |
| 55 Fe | remainder |

|    | Example II | Per cent  |
|----|------------|-----------|
| Cr |            | 20-30     |
| Cu |            | 10-15     |
| Ni |            | 6-10      |
| W  |            | 2-3       |
| Be |            | 8-10      |
| Mo |            | 5-10      |
| Al |            | 2-3       |
| C  |            | 2½-3      |
| Fe |            | remainder |

|    | Example III | Per cent  |
|----|-------------|-----------|
| Cr |             | 20-25     |
| Cu |             | 10-15     |
| Ni |             | 6-10      |
| W  |             | 3-5       |
| B  |             | 3-4       |
| Al |             | 2-3       |
| Mo |             | 10-12     |
| C  |             | 2½-3      |
| Fe |             | remainder |

|    | Example IV | Per cent  |
|----|------------|-----------|
| Cr |            | 20-30     |
| Cu |            | 10-15     |
| Ni |            | 6-15      |
| W  |            | 5-6       |
| Mo |            | 15-18     |
| Al |            | 2-3       |
| Ti |            | 1-2       |
| C  |            | 2½-3      |
| Fe |            | remainder |

The process of manufacturing the pre-alloy is the same as that of the alloy in application 553681, now Patent No. 1,890,540, Dec. 13, 1932: white special pig iron, practically free from phosphorus, sulphur, silicon and manganese is melted together with a high-percentage ferro-chromium, a high-percentage ferro-tungsten, purest nickel and partially refined copper or copper-aluminium respectively. Added to this are, as the case may be, the required quantity of the further refining metals: zirconium, aluminium, boron, beryllium, molybdenum and titanium. The mixture is then thoroughly melted in a covered and strongly heated crucible of graphite, the slag layer is then removed, and the melt is, if necessary, well stirred and then cast in moist sand in simple moulds and is made to solidify as quickly as possible. In this way are obtained the alloys of a ledeburitic structure, in which now also the carbon is present as a carbide-combination, so that the alloys are free from graphite.

110

105

90

95

100

The pre-alloys serve, in the first line, for producing steels practically free from silicon. By using the new alloys as a pre-alloy for manufacturing special steels practically free from silicon, the valuable advantage is obtained that it becomes possible to add to the steel also the highly combustible refining metals: zirconium, aluminum, boron, beryllium, molybdenum and titanium, without causing any losses. The substance <sup>5</sup> <sup>10</sup> position of the finished steel is not within the scope of the invention.

We claim:

1. A ledeburitic pre-alloy free from graphite for manufacturing steels containing carbon, chromium, tungsten, nickel, copper and iron, said pre-alloy containing approximately the following main constituents: 20 to 30% chromium, 2 to 6% tungsten, 6 to 15% nickel, 10 to 15% copper, 2½ to 3% carbon; and of auxiliary constituents consisting of <sup>15</sup> <sup>20</sup> 5 to 18% molybdenum and the balance substantially iron and impurities.

2. A pre-alloy free from graphite intended for use in the manufacture of steels containing carbon, chromium, tungsten, nickel, copper and iron, said pre-alloy containing approximately the following main constituents: 20 to 30% chromium, 10 to 15% copper, 6 to 10% nickel, 2 to 3% tungsten and 2½ to 3% carbon; and auxiliary constituents consisting of 5 to 8% zirconium and 6 to 12% molybdenum and the balance substantially iron. <sup>85</sup>

3. A pre-alloy free from graphite intended for use in the manufacture of steels containing carbon, chromium, tungsten, nickel, copper and iron, said pre-alloy containing approximately the following main constituents: 20 to 30% chromium, 10 to 15% copper, 6 to 10% nickel, 2 to 3% tungsten and 2½ to 3% carbon; and auxiliary constituents consisting of 15 to 18% molybdenum and 1 to 2% titanium and the balance substantially iron. <sup>90</sup>

JOSEPH NOVAK. <sup>95</sup>  
ROMAN KESSELRING.

25

100

30

105

110

115

120

125

130

135

140

145

150